# EUROPEAN PATENT SPECIFICATION

(11) **EP 3 126 552 B1**
(45) Date of publication and mention of the grant of the patent: **21.03.2018**
(21) Application number: 15724103.5
(22) Date of filing: 25.03.2015
(51) Int. Cl.: D01D 13/00, D01F 6/92, D01D 5/16, D01D 10/02

(54) **A SYSTEM FOR INDUSTRIAL YARN PRODUCTION FROM COMPOSITE POLYETHYLENE NAPHTHALATE MATERIAL**
SYSTEM ZUR INDUSTRIELLEN GARNHERSTELLUNG AUS VERBUNDSTOFFPOLYETHYLEN-NAPHTHALAT-MATERIAL
SYSTÈME POUR LA PRODUCTION DE FIL INDUSTRIEL À PARTIR DE MATÉRIAU COMPOSITE À BASE DE POLYÉTHYLÈNE NAPHTALATE

(30) Priority: 01.04.2014 TR 201403779
(43) Date of publication of application: 08.02.2017
(73) Proprietor: Kordsa Teknik Tekstil A.S, Izmit / Kocaeli (TR)
(72) Inventor: GUVEN, Emine, 41310 Kocaeli (TR); TURKARSLAN, Ozlem, 41310 Kocaeli (TR)
(74) Representative: Dericioglu Kurt, Ekin
(86) International application number: PCT/TR2015/000117
(87) International publication number: WO 2015/152844

(56) References cited:
- EP-A1- 0 978 578
- JP-A- 2001 279 533
- US-A- 6 165 614
- KAAN GUNES ET AL: "In situ compatibilization of PEN/LCP blends by ultrasonic extrusion", JOURNAL OF APPLIED POLYMER SCIENCE, vol. 122, no. 1, 5 October 2011 (2011-10-05), pages 354-365, XP055202626, ISSN: 0021-8995, DOI: 10.1002/app.34194

## Description

### Field of the Invention

The present invention relates a system for industrial polyester yarn production, in which the mechanical properties of the yarn (tenacity, modulus, dimensional stability) are improved with additive, in order to be used in industrial fabric production.

### Background of the Invention

Improved mechanical properties and a strong structure are required in conveyor band chafer, membrane and coating fabrics. For such embodiments, processes should be improved without increasing the cost that much, and the resultant fiber should provide high modulus and better dimensional stability compared to the reference. For this reason, studies have been carried out to produce self-reinforced composite PEN yarns.

Liquid Crystal Polymers (LCP), which can be used as reinforcing phase in different polymeric materials, are high performance resins with a unique structure comprising long, hard, rod like high oriented molecules. Rod-like molecules orient themselves in the flow direction during injection or extrusion molding.

The parts molded in LCP exhibit very high dimensional stability even if they are heated up to 200-250°C. Melting temperature of some LCP classes can reach up to 300°C. LCP can generally be used as an additive in many fields depending on its properties. Electronic and electrical components, fuel and gas barrier structures and sensors can be given as example for these fields.

### Summary of the Invention

The objective of the present invention is to provide a system for liquid crystal polymer added industrial polyester yarn production.

Another objective of the present invention is to provide a system for industrial yarn production wherein polyethylene naphthalate is used as polymer.

A further objective of the present invention is to provide a system for industrial yarn production with improved tensile strength and elastic modulus.

### Detailed Description of the Invention

A system for industrial yarn production with LCP added polyethylene naphthalate developed to fulfill the objectives of the present invention is illustrated in the accompanying figure, wherein

Figure 1 is the schematic view of the inventive system for yarn production.

The components shown in Figure 1 are each given with reference numerals as follows:
1. System for industrial yarn production
2. Raw mixture forming unit
   21. Raw particle loading unit
   22. Raw molten extruder
   23. Raw molten cooling unit
3. Primary mixture forming unit
   31. Particle loading and diluting unit
   32. Primary molten extruder
   33. Primary molten cooling unit
4. Primary particle loading unit
5. Extruder
6. Cooling unit
7. Roller
   71. Primary roller
   72. Secondary roller
   73. Tertiary roller
   74. Quaternary roller
8. Hot chamber
   81. First hot chamber
   82. Second hot chamber
9. Winding unit

The inventive system for composite polyethylene naphthalate industrial yarn production system (1) essentially comprises
- at least one raw mixture forming unit (2) wherein the raw polymer particles are prepared,
- at least one primary mixture forming unit (3) wherein the primary polymer mixture is obtained diluting the raw polymer mixture with the main polymer,
- at least one primary particle loading unit (4) wherein the polymer particles forming the primary mixture are filled and heated,
- at least one extruder (5) wherein the primary polymer mixture obtained in primary particle loading unit (4) is melted and spun as filaments with the help of the spinneret located at the exit,
- at least one cooling unit (6) wherein the material coming from the extruder (5) is cooled,
- at least one roller (7) wherein the material is drawn and oriented,
- at least one hot chamber (8) wherein the material is annealed,
- at least one winding unit (9) wherein the material is drawn via the rollers (7) by cooling and heating is wound as yarn.

The raw mixture forming unit (1) present in the inventive system (1) comprises
- at least one raw particle loading unit (21) wherein polyethylene naphthalate (PEN) and liquid crystal polymer (LCP) are mixed,
- at least one raw molten extruder (22) wherein the raw molten mixture is extruded,
- at least one raw molten cooling unit (23) wherein the material going out of the raw molten extruder (22) is cooled.

In the preferred embodiment of the inventive system (1), PEN:LCP ratio of the mixture prepared in the raw particle loading unit (21) is 60:40 by weight. The raw material which is prepared in this ratio and solidified in cooling unit (23) melted and blended in the twin screw extruder (22) is become as particles.

Primary mixture forming unit (3) comprises
- at least one particle loading and diluting unit (31) wherein the polymer particles coming from the raw mixture forming unit (2) are melted and diluted with PEN,
- at least one primary molten extruder (32) wherein the primary raw molten mixture is extruded,
- at least one primary molten cooling unit (33) wherein the material going out of the main molten extruder (32) is cooled.

The raw mixture particles prepared in raw mixture forming unit (2) are sent to the primary molten forming unit (3), and the polymer particles diluted with pure PEN are produced here. The PEN:LCP raw mixture is mixed with PEN till the LCP ratio becomes 1-3% by weight in the particle loading and diluting unit (31). At the said process is preferably carried out at 260-300°C.

In one embodiment of the invention, the molecular weight of the blended polymer particles that are obtained are increased at the outlet of the primary mixture forming unit (3), and their internal viscosity (IV) is increased above 1 dL/g at 240-250°C with solid state polymerization, which takes 12-24 hours. The purpose here is to increase molecular weight to obtain a polymer suitable for yarn drawing by decreasing the degradation and chain movement during extrusion. %Crystallinity increase is above 100% with solid state polymerization.

In one embodiment of the invention, the particles obtained at primary mixture forming unit (3) with increased IV via solid state polymerization are dried in vacuum furnace for at least 24 hours at 120-140°C, and loaded to the primary particle loading unit (4) under nitrogen atmosphere at 120 °C. In order to prevent hydrolytic degradation, the humidity value of the blended and solid state polymerized particles should be under 60 ppm before loading to the extruder (32).

The primary polymer mixture coming out of the primary mixture forming unit (3) is transferred to the primary particle loading unit (4), and dried here at 100-120 °C and sent to the extruder (5) which is heated to 290-320 °C. PEN-LCP polymer mixture comprising 1-3% LCP by weight is become filaments via spinneret at the exit of the extruder (5). In the preferred embodiment of the invention, the length/diameter ratio of the spinneret used at the extruder exit (5) is 2-5, the hole diameter is 1mm. The jet velocity of the material from the extruder (5) is 6-7 m/min, the residence time of the material in the extruder is 11-12 minutes. The throughput here is adjusted as 6-7 g/min.

The PEN-LCP filament coming out of the extruder (5) is transferred to the cooling unit (6) preferably treated with cooling water. In one embodiment of the invention, the length of the cooling unit is 70cm and its temperature is 80-95°C. In the same embodiment of the invention, the distance between the extruder (5) and the cooling unit (6) is adjusted as maximum 10cm. The yarn coming out of the cooling unit (6) first comes to the primary roller (71) and it is sent to the secondary roller (72) from here. In the preferred embodiment of the invention the temperature of the primary roller (71) is between 100-140°C, and the temperature of the secondary roller (72) is between 140-160°C. Cold drawing process is applied on the yarn between these rollers (7).

The yarn coming out of the secondary roller (72) is transferred to the first hot chamber (81) and heated with hot air to 200-250°C here and then transferred to the tertiary roller (73). The temperature of the tertiary roller (73) may vary between 200-250°C. Therefore, hot drawing is performed between the secondary roller (72) and the tertiary roller (73).

The yarn coming out of the tertiary roller (73) enters into the second hot chamber (82) at temperature of 120-180°C. It comes to the quaternary roller (74) which is the last roller without heating, at room temperature; here it is relaxed in ratio of 1-2% and sent to the winding unit (9) in order to be wound.

In the preferred embodiment of the invention, the ratio of the primary roller (71) speed to the extruder (5) exiting speed is between4-6. The ratio of the tertiary roller (73) speed to the primary roller (71) speed may vary between 5-6,5.

When the tenacity and elastic modulus of LCP added PEN yarn in ratio of 1-3% obtained using the inventive system (1) and the yarn manufactured from pure PEN material with the total draw ratio of 6 are compared; the tenacity of the composite yarn produced in the inventive system has increased by 40-45%, and its elastic modulus has increased by 5-10%. When the total draw ratio is more than 6 the tenacity increase is between 25-30%, the elastic modulus improves by 2-5%. When the dimensional stability is considered, the dimensional stability of the 1-3% LCP added PEN yarn is 15-25% better than the pure PEN yarn in 6 drawing ratio.

The conversion ratio is in range of 80-90% when the monofilament yarn which is produced with the inventive system is twisted as 2 layers with 50 twists.

## Claims

1. A system for industrial yarn production from composite polyethylene naphthalate material **comprising**
- at least one raw mixture forming unit (2) wherein the raw polymer particles are prepared,
- at least one primary mixture forming unit (3) wherein the primary polymer mixture is obtained and become particles by using raw polymer particles,
- at least one primary particle loading unit (4) wherein the polymer particles forming the primary mixture are filled and heated,
- at least one extruder (5) wherein the primary polymer mixture obtained in primary particle loading unit (4) are melted and become filaments with the help of the spinneret located at the exit,
- at least one cooling unit (6) wherein the material coming from the extruder (5) is cooled,
- at least one roller (7) wherein the material is drawn and oriented,
- at least one hot chamber (8) wherein the material is annealed,
- at least one winding unit (9) wherein the material is drawn via the rollers (7) by cooling and heating is wound as yarn, and **characterized in that**
- polyethylene naphthalate (PEN) and the liquid crystal polymer (LCP) are mixed in ratio of 60:40 respectively in raw mixture forming unit (2),
- The LCP ratio in the mixture is decreased to 1-3% by weight by diluting the raw mixture with PEN in primary mixture forming unit (3).

2. A system (1) for industrial yarn production from composite polyethylene naphthalate material according to claim 1, **characterized by** raw mixture forming unit (2) which has at least one raw particle loading unit (21) wherein polyethylene naphthalate (PEN) and the liquid crystal polymer (LCP) is mixed by loading in ratio of 60:40 by weight respectively, at least one raw molten extruder (22) wherein raw mixture is melted and extruded;
at least one raw molten cooling unit (23) wherein the material coming out of the raw molten extruder (22) is cooled.

3. A system (1) for industrial yarn production from composite polyethylene naphthalate material according to any one of the preceding claims, **characterized by** primary mixture forming unit (3) which has at least one particle loading and diluting unit (31) wherein the polymer particles coming from the raw mixture forming unit (2) are melted and diluted with PEN such that the LCP ratio will be 1-3% by weight; at least one primary molten extruder (32) wherein the primary raw molten mixture is extruded, at least one primary molten cooling unit (33) wherein the material going out of the main molten extruder (32) is cooled.

4. A system (1) for industrial yarn production from composite polyethylene naphthalate material according to any one of the preceding claims, **characterized by** particle loading and diluting unit (31) wherein PEN is added until the LCP ratio in the mixture is 1-3% by weight the raw PEN-LCP mixture is extruded at 260-300°C.

5. A system (1) for industrial yarn production from composite polyethylene naphthalate material according to any one of the preceding claims, **characterized by** primary particle loading unit (4) wherein the particles obtained at primary mixture forming unit (3) outlet are loaded at nitrogen atmosphere at 120°C after being dried in vacuum furnace for at least 24 hours at 120-140°C.

6. A system (1) for industrial yarn production from composite polyethylene naphthalate material according to any one of the preceding claims, **characterized by** extruder (5) wherein the primary polymer mixture is become filament, and which has a spinneret with length/diameter ratio of 2-5 and the hole diameter is 1mm.

7. A system (1) for industrial yarn production from composite polyethylene naphthalate material according to any one of the preceding claims, **characterized by** extruder (5) wherein the jet velocity of the polymer mixture as filament is 6-7 m/min.

8. A system (1) for industrial yarn production from composite polyethylene naphthalate material according to any one of the preceding claims, **characterized by** extruder (5) wherein the throughput of the polymer mixture as filament is adjusted as 6-7 g/min.

9. A system (1) for industrial yarn production from composite polyethylene naphthalate material according to any one of the preceding claims, **characterized by** cooling unit (6) wherein the filament coming out of the extruder (5) is cooled with cooling water at 80-95°C.

10. A system (1) for industrial yarn production from composite polyethylene naphthalate material according to any one of the preceding claims, **characterized by** primary roller (71) to which the filament coming out of the cooling unit (6) is transferred, at temperature of 100-140°C.

11. A system (1) for industrial yarn production from composite polyethylene naphthalate material according to any one of the preceding claims, **characterized by** the secondary roller (72) at temperature of 140-160°C to which the filament coming out of the primary roller (71) is transferred and wherein cold drawing is applied on the filament.

12. A system (1) for industrial yarn production from composite polyethylene naphthalate material according to any one of the preceding claims, **characterized by** first hot chamber (81) to which the filament coming out of the secondary roller (72) is transferred and in which it is used with hot air at temperature of 200-250°C.

13. A system (1) for industrial yarn production from composite polyethylene naphthalate material according to any one of the preceding claims, **characterized by** the tertiary roller (73) at temperature of 200-250°C to which the filament coming out of the first hot chamber (81) is transferred and wherein hot drawing is applied on the filament.

14. A system (1) for industrial yarn production from composite polyethylene naphthalate material according to any one of the preceding claims, **characterized by** second hot chamber (82) at temperature of 120-180°C to which the filament coming out of the tertiary roller (73) is transferred.

15. A system (1) for industrial yarn production from composite polyethylene naphthalate material according to any one of the preceding claims, **characterized by** the quaternary roller (74) without heating to which the filament coming out of the second hot chamber (82) is transferred and wherein hot drawing is applied on the filament.

16. A system (1) for industrial yarn production from composite polyethylene naphthalate material according to any one of the preceding claims, **characterized by** winding unit (9) wherein the filament coming out of the quaternary roller (74) is wound as yarn by relaxing 1-2%.

## Patentansprüche

1. Ein System zur industriellen Garnherstellung aus zusammengesetztem Polyethylennaphthalat-Material **aufweisend**
- mindestens eine Rohmischung bildende Einheit (2), in der die Rohpolymerpartikel hergestellt sind,
- mindestens eine primäre Mischung bildende Einheit (3), wobei die primäre Polymermischung erhalten und zu Partikeln werden, indem rohen Polymerpartikel verwendet sind,
- mindestens eine primäre Partikelladeeinheit (4), wobei die die primäre Mischung bildende Polymerpartikeln gefüllt und erhitzt werden,
- mindestens einen Extruder (5), in dem die primäre Polymermischung, das in der primären Partikelladeeinheit (4) erhalten wird, geschmolzen sind und mit Hilfe der Spinndüse, die sich am Austritt befindet, zu Filamenten wird,
- mindestens eine Kühleinrichtung (6), in der das Material aus dem Extruder (5) gekühlt wird,
- mindestens einen Roller (7), in dem das Material gezogen und orientiert wird,
- mindestens eine heiße Kammer (8), in der das Material geglüht wird,
- mindestens eine Wickeleinrichtung (9), in der das Material mittels eines Rollers (7) durch Kühlen gezogen wird und die Hitze als Garn aufgewickelt wird, und **dadurch gekennzeichnet, dass**
- Polyethylennaphthalat (PEN) und das Flüssigkristallpolymer (LCP) werden jeweils in einem Verhältnis von 60: 40 in der Rohmischung bildenden Einheit (2) gemischt,
- Das LCP- Verhältnis in der Mischung wird auf 1-3 Gew.- % reduziert, indem die Rohmischung mit PEN in der primäre Mischung bildenden Einheit (3) verdünnt wird.

2. Ein System (1) für industrielle Garnherstellung aus zusammengesetztem Polyethylennaphthalat-Material nach Anspruch 1, **gekennzeichnet durch** eine Rohmischung bildende Einheit (2), die mindestens eine Rohpartikel-Ladeeinheit (21) aufweist, wobei Polyethylennaphthalat (PEN) und das Flüssigkristallpolymer (LCP) durch Beladung im Gewichtsverhältnis von jeweils 60:40 gemischt werden, mindestens ein roher geschmolzener Extruder (22), wobei die Rohmischung geschmolzen und extrudiert wird;
mindestens eine rohe geschmolzene Kühleinheit (23), wobei das Material, das aus dem rohen geschmolzenen Extruder (22) austritt, gekühlt wird.

3. Ein System (1) für industrielle Garnherstellung aus zusammengesetztem Polyethylennaphthalat-Material nach einem der vorangehenden Ansprüche, **gekennzeichnet durch** eine primäre Mischung bildende Einheit (3), die mindestens eine Partikellade- und Verdünnungseinheit (31) aufweist, wobei die aus der Rohmischung bildenden Einheit (2) austretende Polymerpartikel mit PEN so geschmolzen und verdünnt werden, dass das LCP-Verhältnis 1-3 Gew.-% beträgt, mindestens einen primären geschmolzenen Extruder (32), wobei die primäre rohe geschmolzene Mischung extrudiert wird, mindestens eine primäre geschmolzene Kühleinheit (33), wobei das aus dem Hauptschmelzextruder (32) austretende Material gekühlt wird.

4. Ein System (1) für industrielle Garnherstellung aus zusammengesetztem Polyethylennaphthalat-Material nach einem der vorangehenden Ansprüche, **gekennzeichnet durch** einer Partikellade- und Partikelverdünnungseinheit (31), wobei PEN zugegeben wird, bis das LCP-Verhältnis in der Mischung 1 bis 3 Gew.-% beträgt, wobei die PEN-LCP Rohmischung bei 260-300°C extrudiert wird.

5. Ein System (1) für industrielle Garnherstellung aus zusammengesetztem Polyethylennaphthalat-Material nach einem der vorangehenden Ansprüche, **gekennzeichnet durch** eine Partikeladeeinheit (4), die am Auslass der primären Mischung bildenden Einheit (3) erhaltenen Partikel bei 120 °C in Stickstoffatmosphäre geladen werden, nachdem sie mindestens 24 Stunden bei 120 bis 140 °C im Vakuumofen getrocknet wurden.

6. Ein System (1) für industrielle Garnherstellung aus zusammengesetztem Polyethylennaphthalat-Material nach einem der vorangehenden Ansprüche, **gekennzeichnet durch** einen Extruder (5), wobei die Primärpolymermischung zu einem Filament wird und das eine Spinndüse mit einem Länge/ Durchmesser- Verhältnis von 2 bis 5 und einen Lochdurchmesser von 1mm aufweist.

7. Ein System (1) für industrielle Garnherstellung aus zusammengesetztem Polyethylennaphthalat-Material nach einem der vorangehenden Ansprüche, **gekennzeichnet durch** einen Extruder (5), wobei die Strahlgeschwindigkeit der Polymermischung als Filament mit 6 bis 7 g/min eingestellt ist.

8. Ein System (1) für industrielle Garnherstellung aus zusammengesetztem Polyethylennaphthalat-Material nach einem der vorangehenden Ansprüche, **gekennzeichnet durch** einen Extruder (5), wobei der Durchsatz der Polymermischung als Filament mit 6 bis 7 g/min eingestellt wird.

9. Ein System (1) für industrielle Garnherstellung aus zusammengesetztem Polyethylennaphthalat-Material nach einem der vorangehenden Ansprüche, **gekennzeichnet durch** eine Kühleinheit (6), wobei das aus dem Extruder (5) austretende Filament mit einem Kühlungswasser bei 80 bis 95°C gekühlt wird.

10. Ein System (1) für industrielle Garnherstellung aus zusammengesetztem Polyethylennaphthalat-Material nach einem der vorangehenden Ansprüche, **gekennzeichnet durch** Primärroller (71), in den das aus dem Kühleinheit (6) austretende Filament bei einer Temperatur von 100 bis 140°C übertragen wird.

11. Ein System (1) für industrielle Garnherstellung aus zusammengesetztem Polyethylennaphthalat-Material nach einem der vorangehenden Ansprüche, **gekennzeichnet durch** den Sekundärroller (72) bei einer Temperatur von 140 bis 160°C, in den das aus dem Primärroller (71) austretende Filament übertragen wird und in dem Kaltziehen auf dem Filament ausgeübt wird.

12. Ein System (1) für industrielle Garnherstellung aus zusammengesetztem Polyethylennaphthalat-Material nach einem der vorangehenden Ansprüche, **gekennzeichnet durch** eine erste Heißkammer (81), in die das aus der Sekundärroller (72) austretende Filament übertragen wird und in der es mit heißer Luft bei einer Temperatur von 200 bis 250°C verwendet wird.

13. Ein System (1) für industrielle Garnherstellung aus zusammengesetztem Polyethylennaphthalat-Material nach einem der vorangehenden Ansprüche, **gekennzeichnet durch** den Tertiärroller (73) bei einer Temperatur von 200 bis 250°C, zu der das Filament aus der ersten heißen Kammer kommt (81) übertragen wird und wobei Heißziehen auf das Filament ausgeübt wird.

14. Ein System (1) für industrielle Garnherstellung aus zusammengesetztem Polyethylennaphthalat-Material nach einem der vorangehenden Ansprüche, **gekennzeichnet durch** eine zweite Heißkammer (82) bei einer Temperatur von 120 bis 180°C, bis zu der das Filament aus dem Tertiärroller (73) übertragen wird.

15. Ein System (1) für industrielle Garnherstellung aus zusammengesetzten Polyethylennaphthalat-Material nach einem der vorangehenden Ansprüche, **gekennzeichnet durch** den quaternären Roller (74) ohne Erhitzen, auf das der aus der zweiten heißen Kammer (82) kommende Filament übertragen wird und wobei Warmziehen auf das Filament ausgeübt wird.

16. Ein System (1) für industrielle Garnherstellung aus Zusammengesetzen Polyethylennaphthalat-Material nach einem der vorangehenden Ansprüche, **gekennzeichnet durch** eine Wickeleinrichtung (9), in der das Filament, das aus dem quaternären Roller (74) austritt, mit eine Erweiterung von 1-2% als Garn gewickelt wird.

## Revendications

1. Système de production de fil industriel à partir de matériau composite de polyéthylène naphtalate **comprenant**
- au moins une unité de formation de mélange brut (2) dans laquelle les particules de polymère brutes sont préparées,
- au moins une unité de formation de mélange primaire (3) dans laquelle le mélange de polymères primaires est obtenu et devient des particules en utilisant des particules de polymère brutes,
- au moins une unité de chargement de particules primaires (4) dans laquelle les particules de polymère formant le mélange primaire sont remplies et chauffées,
- au moins une extrudeuse (5) dans laquelle le mélange de polymères primaires obtenu dans l'unité de chargement de particules primaires (4) est fondu et devient des filaments à l'aide de la filière située à la sortie,
- au moins une unité de refroidissement (6) dans laquelle le matériau provenant de l'extrudeuse (5) est refroidi,
- au moins un rouleau (7) dans lequel le matériau est étiré et orienté,
- au moins une chambre chaude (8) dans laquelle le matériau est recuit,
- au moins une unité d'enroulement (9) dans laquelle le matériau est tiré par les rouleaux (7) par refroidissement et le chauffage est enroulé en tant que fil, et **caractérisé en ce que**
- le polyéthylène naphtalate (PEN) et le polymère à cristaux liquides (LCP) sont mélangés dans un rapport de 60:40 respectivement dans l'unité de formation de mélange brute (2),
- Le rapport de LCP dans le mélange est réduit à 1-3% en poids en diluant le mélange brut avec du PEN dans l'unité de formation de mélange primaire (3).

2. Système (1) pour la production de fils industriels à partir de matériau composite de polyéthylène naphtalate selon la revendication 1, **caractérisé par** unité de formation de mélange brut (2) qui comporte au moins une unité de chargement de particules brutes (21) dans lequel le polyéthylène naphtalate (PEN) et le polymère à cristaux liquides (LCP) sont mélangés par chargement dans un rapport de 60:40 en poids respectivement, au moins une extrudeuse fondue brute (22) dans laquelle le mélange brut est fondu et extrudé; au moins une unité de refroidissement fondue brute (23) dans laquelle le matériau sortant de l'extrudeuse fondue brute (22) est refroidi.

3. Système (1) pour la production de fils industriels à partir de matériau composite de polyéthylène naphtalate selon l'une quelconque des revendications précédentes, **caractérisé par** unité de formation de mélange primaire (3) qui comporte au moins une unité de chargement et de dilution de particules (31) dans laquelle les particules de polymère provenant de l'unité de formation de mélange brute (2) sont fondues et diluées avec du PEN de sorte que le rapport LCP sera %1-3 par poids; au moins une extrudeuse primaire fondue (32) dans laquelle le mélange primaire brut fondu est extrudé, au moins une unité de refroidissement primaire fondue (33) dans laquelle le matériau sortant de l'extrudeuse principale fondue (32) est refroidi.

4. Système (1) pour la production de fil industriel à partir de matériau composite de polyéthylène naphtalate selon l'une quelconque des revendications précédentes, **caractérisé par** une unité de chargement et de dilution de particules (31) dans laquelle PEN est ajouté jusqu'à ce que le rapport LCP dans le mélange soit de 1-3% poids, le mélange PEN-LCP brut est extrudé à 260-300°C.

5. Système (1) pour la production de fils industriels à partir de matériau composite de polyéthylène naphtalate selon l'une quelconque des revendications précédentes, **caractérisé par** une unité de chargement de particules primaires (4) dans laquelle les particules obtenues à la sortie de l'unité de formation de mélange primaire (3) sont chargées à 120°C après avoir été séchées dans un four sous vide pendant au moins 24 heures à 120-140°C.

6. Système (1) pour la production de fils industriels à partir de matériau composite de polyéthylène naphtalate selon l'une quelconque des revendications précédentes, **caractérisé par** une extrudeuse (5) dans laquelle le mélange de polymère primaire est devenu un filament, et qui a une filière avec un rapport longueur / diamètre de 2 à 5 et le diamètre du trou est de 1 mm.

7. Système (1) pour la production de fils industriels à partir de matériau composite de polyéthylène naphtalate selon l'une quelconque des revendications précédentes, **caractérisé par** extrudeuse (5) dans laquelle la vitesse du jet du mélange de polymères sous forme de filament est de 6-7 m / min.

8. Système (1) pour la production de fils industriels à partir de matériau composite de polyéthylène naphtalate selon l'une quelconque des revendications précédentes, **caractérisé par** extrudeuse (5) dans laquelle le débit du mélange de polymères sous la forme d'un filament est ajusté à 6-7 g / min.

9. Système (1) pour la production de fils industriels à partir de matériau composite de polyéthylène naphtalate selon l'une quelconque des revendications précédentes, **caractérisé par** unité de refroidissement (6) dans laquelle le fil sortant de l'extrudeuse (5) est refroidi avec de l'eau de refroidissement à 80-95 °C.

10. Système (1) pour la production de fils industriels à partir de matériau composite de polyéthylène naphtalate selon l'une quelconque des revendications précédentes, **caractérisé par** le rouleau primaire (71) auquel le fil sortant de l'unité de refroidissement (6) est transféré, à une température de 100-140°C.

11. Système (1) pour la production de fils industriels à partir de matériau composite de polyéthylène naphtalate selon l'une quelconque des revendications précédentes, **caractérisé par** le rouleau secondaire (72) à une température de 140-160°C à laquelle le fil sortant du rouleau primaire (71) est transféré et dans lequel un étirage à froid est appliqué sur le filament.

12. Système (1) pour la production de fils industriels à partir de matériau composite de polyéthylène naphtalate selon l'une quelconque des revendications précédentes, **caractérisé par** la première chambre chaude (81) à laquelle est transféré le filament sortant du rouleau secondaire (72) et dans laquelle il est utilisé avec de l'air chaud à une température de 200-250°C.

13. Système (1) pour la production de fils industriels à partir de matériau composite de polyéthylène naphtalate selon l'une quelconque des revendications précédentes, **caractérisé par** le rouleau tertiaire (73) à une température de 200-250°C à laquelle est transféré le filament sortant de la première chambre chaude (81) et dans lequel un étirage à chaud est appliqué sur le filament.

14. Système (1) pour la production de fils industriels à partir de matériau composite de polyéthylène naphtalate selon l'une quelconque des revendications précédentes, **caractérisé par** une seconde chambre chaude (82) à une température de 120-180°C à laquelle est transféré le filament sortant du rouleau tertiaire (73).

15. Système (1) pour la production de fils industriels à partir de matériau composite de polyéthylène naphtalate selon l'une quelconque des revendications précédentes, **caractérisé par** le rouleau quaternaire (74) sans chauffage auquel le filament sortant de la deuxième chambre chaude (82) est transféré et dans lequel un étirage à chaud est appliqué sur le filament.

16. Système (1) pour la production de fils industriels à partir de matériau composite de polyéthylène naphtalate selon l'une quelconque des revendications précédentes, **caractérisé par** une unité d'enroulement (9) dans laquelle le fil sortant du cylindre tertiaire (74) est enroulé en tant que fil en relaxant 1-2%.
